

Aug. 14, 1951

C. C. VERHEYEN

2,564,136

CORUNDUM CRYSTAL RECORDING OR REPRODUCING MEMBER

Filed July 2, 1946

Fig. 1



Fig. 4

Fig. 2

Fig. 3

INVENTOR.

COENRAAD C. VERHEYEN

BY

AGENT

## UNITED STATES PATENT OFFICE

2,564,136

CORUNDUM CRYSTAL RECORDING OR  
REPRODUCING MEMBER

Coenraad Cornelis Verheyen, Eindhoven, Netherlands, assignor to Hartford National Bank and Trust Company, Hartford, Conn., as trustee

Application July 2, 1946, Serial No. 680,910  
In the Netherlands March 4, 1943Section 1, Public Law 690, August 8, 1946  
Patent expires March 4, 1963

3 Claims. (Cl. 274—38)

1

The invention relates generally to cutting members for mechanically recording or reproducing records, such as phonograph records, for example, and more particularly to those members, which consists of a crystal.

In recording sound with the aid of such a cutting member which is made, for example, of corundum crystal and which has a V-shaped cutting edge, there arises the drawback that the cutting edges wear off very soon or that small pieces of crystal break off therefrom, with the result that, for example, sound tracks recorded with the aid of such a member have, during reproduction, a kind of fading effect with distortion. As regards members with the aid of which, for example, mechanically provided sound tracks are reproduced, the above-mentioned drawback results in that the oscillation tracks wear off or are damaged more rapidly than usual.

With the member according to the invention, this drawback is avoided due to the fact that the longitudinal axis of the member and the principal axis of the crystal are perpendicular to one another, which may be achieved by a properly chosen method of grinding. It has been found that in this case the highest resistance is opposed against wear and crumbling off.

The invention will be explained more fully, by way of example, with reference to the accompanying drawing.

Fig. 1 represents diagrammatically a corundum crystal wherein A—A represents the principal axis.

The Figs. 2 and 3 represent diagrammatically a rear-view and a side-view respectively of a recording chisel of known type which has an obtuse vertical angle. B—B is the longitudinal axis. During the grinding operation care is taken to achieve that the axis B—B will be perpendicular to the axis A—A.

Fig. 4 represents part of a phonograph needle wherein B—B also represents the longitudinal axis.

What I claim is:

1. A member for mechanically recording or reproducing phonograph records comprising a uniaxial corundum crystal, said member having the longitudinal axis thereof perpendicular to the principal axis of said crystal said member

2

having a pair of side surfaces each substantially parallel to said longitudinal axis and another pair of surfaces at one end thereof each extending from one of said side surfaces, respectively, at a substantial angle to said longitudinal axis and intersecting with each other to form a substantially sharp edge at said one end thereof.

2. A member for mechanically recording or reproducing phonograph records comprising a crystal having only one principal axis, said member having the longitudinal axis thereof perpendicular to said principal axis of said crystal, said member having a pair of side surfaces each substantially parallel to said longitudinal axis and another surface at one end thereof extending from one of said side surfaces at a substantial angle to said longitudinal axis and terminating to form a substantially sharp edge at said one end thereof.

3. A member for mechanically recording or reproducing phonograph records comprising a crystal having only one principal axis, said member having the longitudinal axis thereof perpendicular to said principal axis of said crystal, said member having a pair of side surfaces each substantially parallel to said longitudinal axis and another pair of surfaces at one end thereof each extending from one of said side surfaces, respectively, at a substantial angle to said longitudinal axis and intersecting with each other to form a substantially sharp edge at said one end thereof.

COENRAAD CORNELIS VERHEYEN.

## REFERENCES CITED

35 The following references are of record in the file of this patent:

## UNITED STATES PATENTS

| Number    | Name    | Date          |
|-----------|---------|---------------|
| 484,583   | Edison  | Oct. 18, 1922 |
| 1,737,253 | Linsell | Nov. 26, 1929 |
| 2,355,877 | Le Van  | Aug. 15, 1944 |

## FOREIGN PATENTS

| Number  | Country | Date          |
|---------|---------|---------------|
| 402,575 | France  | Oct. 12, 1902 |
| 728,644 | France  | Apr. 18, 1932 |
| 751,047 | France  | June 12, 1933 |